

J. McF. SYLVESTER.

TUBULAR FORGING AND PROCESS FOR MAKING THE SAME.  
APPLICATION FILED AUG. 12, 1920.

1,437,690.

Patented Dec. 5, 1922.



Inventor

John M. Sylvester,

By Watson, Foit, Morse & Grindle,

Attorneys.

Patented Dec. 5, 1922.

1,437,690

# UNITED STATES PATENT OFFICE.

JOHN MCFALL SYLVESTER, OF ROSEMONT, PENNSYLVANIA, ASSIGNOR TO BETHLEHEM STEEL COMPANY, OF BETHLEHEM, PENNSYLVANIA, A CORPORATION OF PENNSYLVANIA.

## TUBULAR FORGING AND PROCESS FOR MAKING THE SAME.

Application filed August 12, 1920. Serial No. 402,957.

To all whom it may concern:

Be it known that I, JOHN MCFALL SYLVESTER, a citizen of the United States, and residing at Rosemont, Lehigh County, State of Pennsylvania, have invented certain new and useful Improvements in Tubular Forgings and Processes for Making the Same, of which the following is a specification.

My invention relates to an improved process of making tubular steel forgings of large diameter with relatively thin walls and to the article produced thereby. It has reference particularly to the manufacture of tubular forgings used in making air-flasks for naval torpedoes.

My invention finds its particular value and utility in the production of large tubular steel forgings with relatively thin walls having an outside diameter of at least 18 inches and a length of not less than six feet. It will be described with special reference to the manufacture of a 21" naval torpedo air-flask forging, which forgings have an outside diameter of about 22 inches and a length of about 13 feet and walls approximately  $2\frac{1}{4}$ " thick.

In the processes heretofore employed for the manufacture of naval torpedo air-flask forgings, considerable loss and waste of material results. In one of such prior processes a cylindrical steel ingot is cast and after certain parts are cut away to remove the defective material produced in casting, the ingot is bored longitudinally of its axis and the resultant tubular blank is forged and worked in sections by hammer or press, the sections being heated prior to each forging operation. The finished forging is then rough machined to the required dimensions.

In the case of a 21" naval torpedo air flask forging, this process results in the production of a rough machined forging weighing about 2700 lbs. from an original ingot weighing approximately 22,500 lbs., or a net yield in finished product of only 12% of the original weight of material employed.

In another process a rectangular steel ingot is cast and rolled into the form of a rectangular plate which, after certain parts are discarded, is sheared into two portions, each of which is then cross-rolled into an approximately square plate. From each of these plates a circular blank is cut and such blanks are then dished or cupped and drawn

through dies to produce the desired tubular 55 forging. In order to cup the circular blanks and draw them into final form, this process requires repeated passage of the blanks through dies and the use of punches of different diameter in the various passes. Ap- 60 proximately eleven passes are necessary, and repeated reheating of the forging is also re- 65 quired. In the case of 21" naval air-flask forgings this process has been found to re- 70 sult in the production of two forgings of 2700 lbs. each from an original ingot of ap- 75 proximately 34,000 lbs., or a net yield of only about 16%.

In both of the processes above described much loss of material therefore occurs by 70 the fact that portions of the ingot or blank must be bored or cut away causing unavoidable loss of material and further loss is occasioned by the formation of scale during the repeated heatings to which the forging 75 must be subjected. Such scale must be removed to obtain a perfect product which is difficult to accomplish where numerous re- 80 heatings are necessary with the result that considerable scale finds its way into the fin- 85 ish product causing the formation of forgings which are defective and lack uniform- 90 ity. Furthermore, defects such as "spurs", "cold shuts", "laps", etc., are common in 95 forgings produced in the hammer or press forging process, while "laminations" are common in forgings produced by the rolling process. And in addition to the foregoing 100 defects, it is found that repeated reheating, necessary in prior processes, increases the percentage of unacceptable product on account of overheating or underheating which are apt to occur and in general by working the metal at improper temperatures.

By the process of my invention no cutting 95 away of the metal is necessary, except the material usually discarded from the cast ingot, and only a limited number of re- 100 heatings is required, with the result that a forging of a given weight can be pro- 105 duced from a much smaller ingot of metal than is possible with the former processes referred to. By my process I am able to obtain in the case of a 21" naval torpedo air-flask forging, a finished forging weigh- 110 ing approximately 2700 lbs. from an ingot weighing 10,500 lbs., which represents a net yield of approximately 26% as com-

pared with 12% and 16% obtained by former processes. Forgings can therefore be produced according to my invention more cheaply and economically since smaller 5 ingots may be employed to produce forgings of a given weight.

Furthermore, it has been found that tubular forgings produced according to my invention possess few if any of the defects due 10 to the presence of scale and that they are uniformly free from defects such as "spurs", "cold shuts", "laps" and "laminations." And in addition to being free from such defects, these forgings, as will later appear, 15 possess qualities much superior to those produced by former processes.

In the drawings accompanying this specification and forming a part thereof, I have illustrated in a diagrammatic way the operations involved in producing a torpedo air-flask forging according to my improved process.

Referring to the drawings in detail:

Figure 1 illustrates an ingot of metal 25 from which the forging is to be made;

Figure 2 shows the ingot with the upper portion of the same cut away to eliminate defective material;

Figure 3 illustrates diagrammatically the 30 operation of upsetting the ingot;

Figure 4 illustrates in a more or less diagrammatic way the operation of partially piercing the ingot;

Figure 5 is a diagrammatic view showing 35 a step in the operations of drawing the ingot after it has been subjected to the operations previously referred to; and

Figure 6 is a view similar to Figure 5 illustrating a further step in the drawing 40 operation.

In the practice of my invention as applied to the production of a naval torpedo air-flask forging, I first cast a steel ingot from metal having approximately the following 45 chemical composition:

|  | Mn.        | P.          | S.   | Ni.  | Cr.         | Si.              |
|--|------------|-------------|------|------|-------------|------------------|
|  | 25 to .55% | .15 to .50% | .05% | .04% | 1.0 to 3.0% | .60 to 2.0% .20% |

In producing air-flask forgings of the kind mentioned, it is necessary to cast an 50 ingot approximately 30" in diameter and weighing approximately 10,500 pounds, and I prefer to use for that purpose an iron mold. Heretofore, cylindrical ingots of more than 20" in diameter have never 55 been cast in an iron mold and it has been thought impracticable or impossible to cast ingots of that size in such a mold. However, I have found that this can be done by 60 pouring the metal at a slow rate and by employing molds having extremely thick walls at the bottom, tapering to thinner walls at the top and by using a stool having a deep concave portion. Cylindrical ingots so cast are particularly adapted for the subsequent operations of my process. The term

cylindrical as used herein is intended to include ingots having a slight taper as well as those of true cylindrical form.

In practicing my invention ingots may be used in which the exterior surface is provided with flutes or corrugations but forgings made from such ingots are not as satisfactory as those made from cylindrical ingots. This is due to the fact that in the upsetting and piercing operations herein-after described difficulty is experienced in filling out the die. The metal at the root of the corrugations is thus worked less than other portions which results in lack of uniformity in the metal of the forging. Ingots 70 cast in sand or in sand-lined molds also may be employed but such ingots are apt to be contaminated by the presence of sand and are frequently defective due to segregated streaks caused by slow rate of cooling, 75 and ingots so cast are not therefore as satisfactory for my process as ingots cast in iron.

In carrying out my process, the ingot is cast with a cylindrical body and with a cone-shaped part A', (Figure 1), which is generally known as the "hot top". After casting, a top portion of about 20%, approximately the weight of the "hot top", is discarded to eliminate defective metal produced in the casting operation, leaving a 80 cylindrical ingot B as shown in Figure 2 of the drawing.

After the discard is cut therefrom the ingot B is reheated to a temperature from 900° C. to 1200° C. and it is then placed in 100 a die illustrated at C in Figure 3 which is somewhat larger in diameter than the diameter of the ingot as will appear from the dotted lines in said figure, such dotted lines representing the size of the ingot before further treatment. The inner wall of the die while approximately cylindrical in shape tapers slightly, the greater diameter being at the top. While in the die C the ingot is compressed or upset by means of a flat punch 105 D which is operated from any suitable source of power such as a hydraulic press. The diameter of the punch D is slightly less than the top diameter of the die. It will be understood that after the upsetting operation is completed the ingot is enlarged radially so that it assumes the shape of the die 115 C as shown by the solid lines in said Figure 3. This upsetting operation refines and compresses and densifies the metal to a considerable extent and improves its structure so that in the subsequent operations of drawing the metal, the development of defects on the surface of the forging is largely prevented.

While the ingot is still confined in the die C and preferably without being reheated, it is partially pierced by a piercing punch E as diagrammatically illustrated in Figure 4 of the drawing, this punch being slightly 120

tapered. The punch E is also operated by a hydraulic press or from any other suitable source of power. The ingot is pierced to such a depth as to leave a bottom disc F in 5 the ingot of sufficient thickness to withstand the pressure exerted thereon by the drawing punch during the drawing operations hereinafter described.

The operation of piercing the ingot causes 10 the metal to flow in a direction generally opposite to the direction of travel of the punch as shown at G in Figure 4, and in addition to partially piercing the ingot, this operation further works the inner and outer 15 surfaces of the pierced ingot and also materially compresses, works and refines the crystalline structure of the metal throughout the ingot.

The operation of piercing the ingot produces 20 what will hereinafter be termed a cupped blank, this blank in the case of air-flask forgings having an internal diameter of approximately 16" and a cylindrical wall approximately 6 $\frac{1}{4}$ " thick.

25 The cupped blank is now removed from the die slightly reheated, preferably to a temperature from 900° to 1200° C. and is placed on a punch H of a draw bench diagrammatically illustrated in Figure 5 of 30 the drawing. The cradle of the draw bench has three or four circular dies I centered on the path of the axis of the punch H, each successive die being of smaller diameter than the preceding one. In the case of air-flask 35 forgings, the stroke of the punch should be approximately 35 feet. The cupped blank is passed through all the dies of the series, each die in turn reducing the overall diameter of the blank. The blank is again 40 slightly reheated and given a pass through a second set of circular dies of smaller diameter than those of the first set and after being again reheated, it is passed through a third set of dies smaller in diameter than 45 those of the second set. Each successive die in the second and third sets is also preferably smaller than the preceding die.

A single draw punch H may be used for the three sets of dies, this punch being 50 slightly tapered to facilitate stripping and the diameter and taper thereof being substantially the same as the taper and diameter of the piercing punch E heretofore described. The draw punch is preferably provided with means for stripping the blank 55 from the punch and the blank is stripped after each drawing operation. After the third pass through the drawing dies, the bottom disc F is discarded and the resulting tube is rough machined to the required 60 dimensions, giving as heretofore noted, a rough machined 21" naval torpedo air-flask forging weighing approximately 2700 lbs. from an ingot weighing 10,500 lbs. or a net 65 yield of approximately 26%.

During the foregoing drawing operations the cylindrical wall of the blank, in the case of torpedo air-flask forgings, is reduced from a thickness of approximately 6 $\frac{1}{2}$ " to a thickness of approximately 2 $\frac{3}{4}$ ". 70 The entrance angle of the drawing dies, which is about 12°, is designed to radially forge the wall of the blank and effect elongation without stretching the metal beyond its elastic limit. Such drawing operations, 75 together with the previous treatment to which the metal has been subjected greatly improves its physical properties and produces a product much superior to that secured by any other process at present known 80 to the art. These operations result in working the metal so that the same is compressed and refined and densified throughout resulting in a forging having a uniform grain and a compact, homogeneous structure 85 throughout, and which is practically free from the defects found in forgings produced by prior processes. My process therefore results in a superior product and at the same time requires less metal to produce 90 a forging of a given weight.

The requirements for naval torpedo air-flask forgings are exceedingly rigid and heretofore great difficulty has been experienced by manufacturers in producing forgings of sufficient strength and uniformity of structure to meet such requirements. A very high percentage of such forgings have heretofore been rejected by the Government because of their failure to meet the standard 100 required. With my process such difficulty is practically obviated. The forgings made by this process possess properties which fully meet the Government requirements and practically one hundred per cent of the forgings thus made are found to be acceptable. 105

While the invention has been described with special reference to the production of naval torpedo air-flask forgings, it is obviously applicable for the production of large 110 size tubular forgings for any purpose and it is not therefore intended to limit the invention to forgings adapted for use as air-flasks for torpedoes.

Having thus described my invention what 115 I claim as new and desire to secure by Letters Patent is:

1. A process of making torpedo air flask forgings which consists of the following operations substantially as described, upsetting 120 a cylindrical ingot in a confining die, partially piercing said ingot to form a cupped blank, drawing said blank through a series of dies, thereby reducing its overall diameter, all of said operations being performed 125 while the metal is in a heated condition.

2. A process of making naval torpedo air-flask forgings consisting in confining a solid cylindrical ingot of steel in a die closely surrounding the same, forcing a plunger into 130

said die to partially pierce the ingot and form a cupped blank and drawing said blank through order dies to elongate the same.

5 3. A torpedo air flask forging made by casting a cylindrical ingot, partially piercing the same to form a blank and drawing the blank through a series of dies to reduce its overall diameter.

10 4. A torpedo air flask forging made by upsetting a cylindrical ingot in a confining die, partially piercing the ingot to form a

cupped blank and drawing the blank through a series of dies to reduce its overall diameter.

15

5. A torpedo air flask forging more than 18 inches in diameter with relatively thin walls made by upsetting a cylindrical ingot in a confining die, partially piercing the ingot to form a cupped blank and drawing the blank through a series of dies to reduce its overall diameter.

In testimony whereof I affix my signature.  
JOHN McFALL SYLVESTER,